

# UNITED STATES PATENT OFFICE.

FRANK A. PALEN, OF NEW YORK, N. Y.

## PROCESS FOR THE SCIENTIFIC CURING OF WOODS.

1,066,523.

Specification of Letters Patent.

Patented July 8, 1913.

No Drawing.

Application filed November 20, 1911. Serial No. 661,394.

To all whom it may concern:

Be it known that I, FRANK A. PALEN, a citizen of the United States, residing at New York, in the county of New York and State of New York, have invented certain new and useful Improvements in Processes for the Scientific Curing of Woods, of which the following is a specification.

An object of my invention is to provide an improved process whereby an efficient preservation can be obtained uniformly throughout the entire thickness of the wood, without injurious checking or disruption of the wood fibers.

15 A further object of my invention is to provide an improved process, by which the thoroughly dried and hardened wood fibers will be protected throughout the mass by a coating or varnish of the undecomposed 20 wood resins.

In previous processes for treating woods, the unheated wood has been initially subjected to a vacuum to remove all water and readily volatile aqueous matters, preliminary to treating the wood with heat in the presence of a vacuum. It has been found that such initial vacuum treatment causes localized drying in the outer layers of the wood, whereby said dried outer layers are 25 injuriously checked and disrupted by the heat employed in the succeeding step, and act to retard penetration of the heat to the interior wood layers and to entrap and retain the moisture in said inner layers.

30 In the preferred operation of my invention, the undried wood is placed in a suitable receptacle or retort and subjected to a progressively increasing temperature in the presence of a vacuum of approximately 20" to 28"; the temperature being gradually raised to a maximum preferably below 300° F. and above the point of sterilization. In this step, the gradually increasing temperature causes a progressive penetration of 35 the heat through the entire thickness of the wood, whereby the escape of aqueous vapor from the interior prevents initial drying of the outer wood layers, and enables a thorough drying to be obtained uniformly 40 throughout the wood without injurious checking; thereby placing the wood in condition for insuring hardening of the wood fibers without disruption of the latter and uniform coating of said fibers by the undecomposed wood resins, in the succeeding 45 steps of my process. The vacuum is then

broken and the wood subjected to either dry or moist heat at a temperature below that which would cause decomposition of the wood resins and above the point of sterilization for a sufficient time to produce a substantially uniform temperature throughout the mass of the wood, thereby avoiding injurious fiber strains and warping of the wood and thoroughly hardening the wood 50 fibers. Where moist heat is employed in this step, it can be conveniently provided by admitting steam, preferably superheated, to the retort, or by cutting off the vacuum of the preceding step before complete removal of the aqueous matters has been produced thereby. The wood is then subjected to the combined action of a vacuum of approximately 20" to 28" and dry heat, preferably below 380° F., to cause vaporization 55 of the lighter oils and resins and liquefaction or partial liquefaction of the heavier oils and resins in an undecomposed form and a uniform distribution of said undecomposed resins as an impervious coating 60 or varnish on the sterilized wood fibers throughout the mass.

65 By my above described improved process any possible localization by excessive heating or drying in the outer wood layers 70 is avoided, thereby insuring the necessary uniform drying and heating throughout the mass of the wood to enable a uniform distribution of the undecomposed resins as a protective coating on the wood fibers; there- 75 by eliminating the defects of previous processes, in which uniform distribution of the resins does not always take place and leaves portions of the wood fibers in condition for deterioration under the action of moisture 80 and fungi growths. My invention provides a sterilized homogeneous product, free from 85 weak portions and which efficiently withstands warping and checking under severe 90 climatic conditions.

95 In the foregoing discussion of the operation of my improved process, I have employed the term "resins" or "wood resins" in its broadest sense. It is, of course, obvious that some woods possess practically 100 no resins, but that they have s their equivalent heavy oils of a complex chemical character, and gums of various kinds which act, when liquefied and distributed, as a protective coating for the wood fibers.

I claim:

1: The herein described process of curing

wood, which consists in first subjecting the undried wood to combined action of a vacuum and a progressively increasing temperature, then breaking the vacuum and subjecting the wood to heat alone to produce a substantially uniform temperature throughout the entire mass without decomposition of the wood resins, and then subjecting the wood to the combined action of a vacuum and heat for causing distribution of the wood resins in an undecomposed form.

2. The herein described process of curing wood, which consists in first subjecting the undried wood to the combined action of a vacuum and a progressively increasing temperature raised to a maximum below 300° F., then breaking the vacuum and subjecting the wood to heat alone for a sufficient time to produce throughout the mass of the wood a substantially uniform temperature below the temperature of decomposition of the wood resins, and then subjecting the wood to the combined action of a vacuum and heat for causing distribution of the wood resins in an undecomposed form.

3. The herein described process of curing wood, which consists in first subjecting the undried wood to the combined action of a vacuum and a progressively increasing temperature, then breaking the vacuum and subjecting the wood to heat alone for a sufficient time to produce throughout the mass of the wood a substantially uniform temperature below the temperature of decomposition of the wood resins, and then subjecting the wood to the combined action of a vacuum and heat below a temperature of 380° F.

vacuum and heat below a temperature of 380° F.

4. The herein described process of curing wood, which consists in first subjecting the undried wood to a progressively increasing temperature in the presence of a vacuum, then breaking the vacuum and subjecting the wood to moist heat alone for a sufficient time to produce a substantially uniform temperature throughout the entire mass without decomposition of the wood resins, and then subjecting the wood to the combined action of a vacuum and heat for causing vaporization of the lighter resins and uniform distribution of the heavier wood resins in an undecomposed form.

5. The herein described process of curing wood, which consists in first subjecting the undried wood to the combined action of a vacuum and heat raised progressively to a maximum below 300° F., then breaking the vacuum and subjecting the wood to heat alone for a sufficient time to produce throughout the mass of the wood a uniform temperature below the temperature of decomposition of the wood resins, and then subjecting the wood to the combined action of a vacuum and heat below a temperature of 380° F.

In testimony whereof I affix my signature in presence of two witnesses.

FRANK A. PALEN.

Witnesses:

B. MORFUTT,  
A. B. CHINN.